

## UNITED STATES PATENT OFFICE

1,989,197

## CUP GREASE

William P. Hilliker, Hammond, Ind., assignor to  
 Standard Oil Company, Chicago, Ill., a corpora-  
 tion of Indiana

No Drawing. Application August 9, 1932,  
 Serial No. 628,111

7 Claims. (Cl. 87—9)

This invention relates to lubricants and it per-  
 tains more particularly to that type of a lubri-  
 cant which is generally referred to as cup grease.

Cup greases as a class have one drawback  
 5 which materially limits their applicability and  
 utility. This one material drawback is their lack  
 of stability at high temperatures. If cup greases  
 are used at temperatures of 170—200° F. their  
 10 structure breaks down and the hard soap sepa-  
 rates out, frequently causing feed pipes to become  
 clogged, and/or causing the seizure of bearings or  
 the restriction of free rolling motion of balls or  
 rollers.

The object of my invention is to provide a cup  
 15 grease which will not decompose or separate at  
 these elevated temperatures, particularly in the  
 range of from 170—220° F. A further object is  
 to provide a cup grease which, when it does sepa-  
 rate, yields a soft soap instead of a hard soap,  
 20 thereby insuring continued lubrication and pre-  
 venting seizure of bearings. A further object is  
 to provide a lubricant which can be used where  
 present cup greases are inoperative, particularly  
 25 in hot dispensing systems in the steel industry  
 and in the lubrication of ball bearings. A fur-  
 ther object is to provide an improved method of  
 making greases, to obtain greater uniformity, to  
 decrease the costs, etc.

In practicing my invention I depart from con-  
 30 ventional practice in two important respects.  
 First, I use a different type of calcium soap, one  
 which is more uniform and which yields a re-  
 markably superior product; second, I modify the  
 process of making the lubricant by using a dif-  
 35 ferent order of steps, higher temperatures, and  
 extended period of stirring, etc. The invention  
 will be more clearly understood from the follow-  
 ing detailed description of a preferred embodi-  
 ment.

40 In practicing my invention I may use the fol-  
 lowing formulas:

*Ingredients to make a 100 pound batch of finished  
 cup grease from acid (1) or glyceride (2)*

|                         | (1)     | (2)     |
|-------------------------|---------|---------|
|                         | Pounds  | Pounds  |
| Acid.....               | 14.00   | 14.70   |
| Glyceride.....          |         |         |
| Hydrated lime.....      | 1.80    | 1.80    |
| Caustic soda (dry)..... | 0.20    | 0.20    |
| Water.....              | 1.80    | 2.70    |
| Petroleum oil.....      | 83.70   | 82.05   |
| <i>Analysis</i>         |         |         |
|                         | Percent | Percent |
| Calcium soap.....       | 15.00   | 15.00   |
| Water.....              | 1.30    | 1.30    |
| Glycerine.....          | Trace   | 1.65    |
| Petroleum oil.....      | 83.70   | 82.05   |

The acid and glycerides referred to in this for-  
 60 mula are very different from the fatty acids and

fats usually employed in the manufacture of cup  
 greases. The glycerides are hydrogenated prod-  
 ucts obtained by hydrogenating vegetable or ani-  
 mal oils. Fish oils, cottonseed oils, rapeseed oil,  
 5 corn oil, whale oil, etc. may be hydrogenated in-  
 dividually or in admixture with other oils. I  
 prefer to hydrogenate oils which will yield acids  
 largely of 18 carbon atoms, and these hydro-  
 genated oils are usually made from Menhadin  
 10 oil containing appreciable amounts of cottonseed  
 and/or rapeseed oil. The particular process for  
 hydrogenating the oils and splitting the acids  
 therefrom forms no part of the present invention  
 and will therefore not be described in detail. The  
 15 hydrogenated glyceride and the acid split there-  
 from may be distinguished from natural fats  
 and fatty acids by the relation between their  
 physical and chemical constants such as the titre,  
 iodine number, percent acid, and neutralization  
 20 value. These acids are of the fatty acid type,  
 they are saturated, they contain from C<sub>16</sub> to C<sub>22</sub>  
 chains (structural formula) and their C<sub>16</sub> con-  
 tent is less than 15%. I have found, however,  
 25 that hydrogenated products with specifications  
 closely resembling natural products in these re-  
 spects show a markedly different behavior in cup  
 greases.

In the following specification and claims my  
 improved glycerides will be called hydrogenated  
 fatty oils or hydrogenated fats, and the acids split  
 30 therefrom will be called hydrogenated fatty acid  
 (even though the acid is split from the hydro-  
 genated oil and is not hydrogenated as an acid).

Heretofore cup greases have been prepared by  
 mixing water, oil equivalent in quantity to the  
 fatty acid to be used, and lime, in a steam-  
 jacketed grease mixer. The fatty acid is then  
 added and heat is applied. After an interval of  
 35 about 40 to 60 minutes, when the temperature has  
 reached 240—260° F., the soap is ready for mix-  
 ing. About 2% to 3% of water is added, and  
 when the batch foams up it is driven down by  
 the addition of oil, the heat being abstracted by  
 the addition of cold oil and by the vaporization of  
 40 water so that the temperature drops to about 230°  
 F. Oil is added until the batch contains about  
 25% soap, and during this interval the tempera-  
 ture drops gradually until it reaches about  
 205—210° F. If the desired soap percentage is  
 45 about 15, the batch should reach a tempera-  
 ture of about 180—190° F. at this point. This  
 process is about the same for fats as for fatty  
 acids except that it requires 12 to 20 hours at  
 240—260° F. to effect the saponification of the fats.

Numerous attempts have been made to manu-  
 facture calcium soap greases from commercial  
 stearic acid, oleostearin, etc.—the acids of which  
 have a titre above 48° F., but attempts along this  
 55 line have been unsuccessful. When hydro-  
 genated fats and acids of equivalent titre test are  
 60

employed I have found that much more satisfactory results are obtained. However, the most satisfactory results are accomplished by the use of the following preferred process.

- 5 An amount of oil equal to the amount of fatty acid used is admixed with lime and water in a steam-jacketed mixer, and the hydrogenated fatty acid is mixed therein and heated to about 260° F. Instead of limiting the temperature to 10 260° F., however, I raise the temperature to about 300° F. and I maintain the heating step for a longer interval, usually from an hour to an hour and a half. The batch is then cooled to approximately 240° F., and 1% of water, based on the 15 finished batch, is added. Oil is worked in and the temperature is permitted to drop gradually until at a point of 33% soap a temperature of about 220° F. is reached. The balance of the oil is added while the batch is maintained at a temperature of about 220° F. or slightly above, and during this addition of oil small additions of water, usually about 2%, are added from time to time, depending on the condition of the batch. If a pressure kettle is used, the addition of water 20 25 is not essential, but the mixture should be regulated so that there is always about 1% water on the finished batch.

After all of the oil has been added and the temperature is still up to 220° F., the stirring is continued but the heat turned off—the batch being allowed to drop to a temperature of 190–210° F. If the batch is filled out and run into containers at this point, the finished grease will have a consistency higher than the normal consistency 30 35 for the given soap content but will, on aging, drop in consistency. I prefer to avoid this consistency drop and to maintain a uniform consistency, and I find that this can be accomplished by stirring the batch at 190–210° F. for another 40 hour or hour and a half. The finished grease then has a consistency which is stable against aging.

The temperature during the final grading may be higher than 220° F. without separation, but 45 more frequent additions of water are required at these high temperatures.

It should be understood, of course, that the preferred process hereinabove described is adapted only for use of hydrogenated fats or 50 hydrogenated fatty acids, because if this material is used for naturally occurring fats or fatty acids, such as tallow, lard oil, etc., the batch will separate out into soap and oil at these high temperatures.

- 55 I have made many attempts to prepare cup grease from stearic acid, but in no case have I obtained a grease structure which was stable at these high temperatures. The stearic acid mixtures always break down and give a mixture 60 of hard, soap-oil lumps in oil,—a mixture resembling oil-soaked sawdust. Furthermore, ordinary stearic acid having a titre of about 50 could not even be used in the old process which I referred to above (before describing my improved process). In all cases, the soap will separate and all of the grease maker's tricks to "catch" these batches by the addition of small amounts of fatty acid, etc. are in vain. I am 65 unable to explain why the hydrogenated fats and 70 fatty oils are so radically different from naturally occurring fats and oils in the art of grease making, but the fact remains that this difference is that between success and failure.

Ordinarily cup greases range from about 4% 75 to 35% of soap, and the oil viscosity varies from

about 80 seconds Saybolt at 100° F. to 200 seconds Saybolt at 210° F.—the lower soap-content greases separating at lower temperatures. I have found that greases prepared from hydrogenated fats not only withstand high temperatures, but 5 when they are subjected to extremely high temperatures, such as 260–270° F., and they do separate, the separation is slow and a soap is obtained which is much softer than that which separates from a regular cup grease. This soap-in-oil is really a soap-oil aggregate which separates from the balance of the oil. Apparently 10 in the case of hydrogenated fat greases this aggregate contains a much higher percentage of oil than is usually the case. This is extremely important in actual use, because if a bearing momentarily is heated to a high temperature and hard soap separates out, friction is materially increased which will, in turn, raise the temperature still further, and a complete failure of the 20 grease and bearings results. On the other hand, when the only effect is the separation of a small amount of soft soap, the friction is not materially increased and the bearing recovers as the load is removed. Another feature of my hydrogenated 25 fat or fatty acid cup greases is the fact that the consistency of the grease is greater for a given soap content than when ordinary fats and acids are employed. It should be understood that mica, graphite or other materials may be added 30 to the grease without departing from this invention.

It will be understood that the invention is concerned primarily with calcium soap greases, that if hydrogenated fats are used instead of acids, a 35 longer period of time will be required to make the soap base, that greases of high soap content may be filled at higher temperatures than greases of low soap contents, etc.

While I have described in detail a preferred example of my invention it should be understood that I do not limit myself to the details therein set forth except as defined by the following claims, which should be construed as broadly as the prior art will permit.

I claim:

1. The method of making cup grease which comprises heating a small amount of oil, water and lime with a hydrogenated fatty compound at a temperature of about 260–300° F., for about an hour, cooling the batch to about 240° F., adding small amounts of water with the residual oil until a temperature of about 220° F. is reached, maintaining the temperature at about 220° F. during the addition of the remaining oil, and stirring the finished grease at a temperature of about 190–210° F. for about an hour so that the consistency of the grease will not fall off on aging.

2. The method of making a cup grease which will be stable at temperatures of 170–200° F., which comprises processing oil with a small amount of water and with about 2 to 35% of a calcium soap of a hydrogenated fatty compound by first heating the calcium soap with a small amount of the oil to a temperature of about 260–300° F. and then working in the rest of the oil at a temperature upwards of about 220° F.

3. A cup grease of the class described which comprises about the following formula:

Calcium hydrogenated fatty soap..... 2 to 35%  
Water..... About 0.3 to 1.5%  
Glycerine..... Trace to 4%  
Petroleum oil..... Balance to 100%

4. The method of making a cup grease of im-

proved temperature stability, which comprises heating a small amount of petroleum oil, water and lime with a hydrogenated fatty compound at a temperature of about 260-300° F. until saponification is essentially completed, working in oil and small amounts of water until a soap content of about 2% to 35% is reached, while gradually lowering the temperature of the batch to about 220° F., the amount of water being sufficient to leave about .3% to 1.5% in the finished product, and stirring the batch at a temperature of about 10-30° below the final processing temperature to stabilize the grease against aging.

5. The method of making a cup grease of improved high temperature stability, which comprises processing oil and a small amount of water with about 2% to 35% of a lime soap of a hydrogenated fatty compound having a titre of about 48° F., the oil and lime soap of hydrogenated fatty 10 compound being processed at a temperature above the boiling point of water until all of the oil has been worked in.

6. The method of making a cup grease of improved high temperature stability, which comprises heating substantially equal parts of oil and a hydrogenated fatty acid having a titre of about 48° F. with lime and water at a tempera- 15

ture of about 260-300° F., maintaining said temperature for about an hour to an hour and a half, cooling the mixture to about 240° F., adding about 1% of water based on the finished batch, working in the oil and gradually lowering the temperature until, at a point of about 33% soap, the temperature of about 220° F. is reached, working in the rest of the oil at a temperature of about 220° F., adding small amounts of water so that the finished product will contain about 1% water and about 65-97% oil, and finally stirring the mixture at a temperature below the final processing temperature for stabilizing the grease against aging.

7. An improved cup grease stable for extended periods at a temperature in excess of 190° F. characterized in that it is prepared from the lime soap of a hydrogenated fatty compound, the acids of which have a titre of about 48° F., said cup grease having about the following formula:

|                                 |                       |
|---------------------------------|-----------------------|
| Calcium hydrogenated fatty soap | 2 to 35%              |
| Alkali                          | Substantially neutral |
| Water                           | About 0.3 to 1.5%     |
| Glycerine                       | Trace to 4%           |
| Petroleum oil                   | Balance to 100% 25    |

WILLIAM P. HILLIKER.